

Oct. 13, 1936.

H. A. STAPLES

2,057,454

## METHOD FOR MAKING LEAD SHEATHED CABLES

Filed April 23, 1932

**FIG.1.**



**FIG. 2.**



14 12 INVENTOR  
Horace A. Staples  
BY  
Cooper, Herr & Dunham  
ATTORNEYS

## UNITED STATES PATENT OFFICE

2,057,454

## METHOD FOR MAKING LEAD SHEATHED CABLES

Horace A. Staples, Plainfield, N. J., assignor to  
Habirshaw Cable and Wire Corporation, New  
York, N. Y., a corporation of New York

Application April 23, 1932, Serial No. 607,063

2 Claims. (Cl. 207—10)

The present invention relates to improvements in methods for making electrical cables and more particularly to improved methods for applying metal sheaths to electrical cables to the general end that an improved and more homogeneous and perfect sheath may be produced than heretofore.

More particularly the present invention relates to improvements in the method and machine which forms the subject matter of the copending application of William A. Del Mar and Earle A. Mitchell, Serial No. 601,430, filed March 26, 1932. According to the aforesaid application, provision is made for minimizing the possibility of the introduction of undesired oxide into the sheath of a metal cable as the same is formed from successive metal charges in an extrusion press.

The present invention has for its object the provision of an improved method for making a metal sheath cable wherein a special atmosphere such as a reducing or inert gas is introduced into the extrusion press below the ram as the ram is withdrawn, which special gas atmosphere prevents the formation of undesirable oxide upon the top surface of the preceding metal charge and which special gas atmosphere is also maintained in the metal press during the recharging of the press with a new metal charge so that oxide formation upon the surface of or in the new lead charge is also precluded.

A further object of the present invention resides in the provision of an improved method for lubricating a lead press prior to a charging operation whereby subsequent extrusion operations are facilitated.

A further object of the present invention resides in the provision of an improved method for making lead sheath cable wherein a reducing or inert gas atmosphere together with a quantity of a lubricating medium may be introduced into the lead press cylinder prior to the introduction of a new charge of lead therein, which atmosphere and lubricating medium cooperate to prevent the formation of undesired oxide upon the lead in the cylinder and which lubricating medium also serves to lubricate the walls of the cylinder to facilitate the subsequent extruding operation.

Further and other objects of the present invention will be hereinafter set forth in the accompanying specification and claims and shown in the drawing, which by way of illustration show what I now consider to be a preferred embodiment of the invention.

The drawing shows in Figure 1 the improved machine by which the

present improved method of making a lead sheath cable is carried out; and

Fig. 2 shows a slightly modified construction of ram.

The customary process of applying a lead sheath to a cable comprises the passing of the cable 10 through a closely fitting die 11 which almost abuts another die 12 of a diameter slightly greater than that of the cable. Lead in a hot but solid form is pressed into the space 14 between the two dies and thence into the cylindrical space 15 between the cable and the inside of the larger diameter die. The pressure for extruding the lead sheath is obtained by a hydraulic ram 16 which presses upon a lead charge 17 in the cylinder or lead press chamber 18.

Due to the large amount of lead which has to be used, particularly for a cable of even normal length, it is generally impracticable to perform the extruding operation continuously. It is necessary to stop and re-charge the cylinder 18 from time to time and during these re-charging operations oxide may be formed upon the surface of the old lead charge 17 or in the new lead which is being introduced into the cable or upon the top of the new lead charge. This undesired oxide formation occurs due to the presence of free oxygen in the air in the cylinder and due to the heated condition of the lead. Accordingly, imperfect cables are produced.

In order to prevent the formation of the undesirable oxide, which subsequently becomes introduced into the lead sheath of the cable during the extruding operations, the previous procedure is modified as will now be described.

The ram 16 is provided with a dummy head 22 carried on a stud 23 slidably fitting the head of the ram 16. The stud 23 is interiorly hollowed out as indicated at 24 and from this hollowed out passage in the stud ports or passages 25 extend laterally as shown. The interior of the ram is also provided with a hollowed portion or conduit 26. Connected to the upper portion of the ram and in communication with the conduit portion 26 is a flexible connection 27 which extends to a three-way valve generally designated 28. Beyond the three-way valve 28 is an atomizing device 29 for atomizing a lubricating medium such as oil which is taken into the atomizing device 29 from a reservoir 30. 31 is a pipe or conduit through which a reducing or other inert gas such as illuminating gas, carbon dioxide, steam or the like is supplied under pressure. Such gas free from free oxygen will hereinafter be termed "a special atmosphere".

30

35

40

45

50

55

After one lead charge has been extruded, the plunger or ram head 22 is in contact with the upper surface of the previous lead charge which surface is substantially at the bottom of the cylinder 18. With the ram in lower position, the three-way valve 28 is thrown to a position to admit a mist of lubricating oil and the reducing or other inert gas through the flexible conduit 27 into the interior of the ram. The ram is then raised and the mist of oil and reducing gas is sprayed on the walls of the chamber or lead press cylinder as the ram is withdrawn upwardly. It will be understood that the dummy head 22 on the ram drops and allows the mist to flow laterally to the walls between the upper part of the dummy head and the lower part of the plunger ram. The gas and lubricating medium passes around the dummy head and down into the space between the top of the previous lead charge and the ram, as the ram is withdrawn upwardly. In this way a reducing atmosphere or inert gas atmosphere is maintained in the chamber or space above the old lead charge between the upper surface thereof and the ram as the ram is being withdrawn. The lubricating medium sprays the bore of the lead press with oil, preventing sticking of the ram and facilitating the subsequent extruding operation.

The next step in the operation is to fill the chamber of the metal press cylinder or container with a new charge of metal such as lead. Such metal, for example molten lead, is introduced into the chamber or container of the extrusion press through a removable pipe 32 which leads to a lead pot or lead pump or other source of metal supply. The pipe 32 during the filling operation, is extended down into the special atmosphere in the container. After filling such pipe 32 is removed. During this filling operation the three-way valve 28 is shifted to a position to shut off further supply of gas and lubricating medium and to establish communication between conduit 27 and a pipe 33. Pipe 33 may extend directly to atmosphere or it can extend into a water seal indicated by dotted lines at 34. The lead is then introduced into the chamber and the reducing gas atmosphere is gradually displaced and discharged through pipe 33. During the filling operation it will be appreciated that the reducing gas or other inert atmosphere within the chamber 18 prevents oxidation of the lead either in the new lead charge, which is introduced in a molten state, or upon the top surface of the old lead charge 17. The machine is then ready for the subsequent extruding operation. During the extruding operation the three-way valve is shifted to closed position and extrusion proceeds in the usual manner.

By the above procedure oxygen is prevented from reaching the surface of the old lead charge or the molten lead while such lead is being introduced into chamber 18. The reducing gas or inert gas which was introduced in the chamber or cylinder of the lead press upon upward withdrawal of the ram prevents oxygen from the air from entering the chamber and precludes oxide formation.

Furthermore the lubricating medium supplements the reducing or inert gas upon being highly heated since such lubricating medium under heat itself becomes converted into hydro-carbon gas which has reducing characteristics.

Figure 2 shows a modified form of ram. With this form the supplemental or dummy head 22 is dispensed with and in lieu thereof the ram 16a is so shaped that its lower integral portion constitutes the head. An interior conduit 26a is provided as before and openings or passages 25a extend to the periphery of the ram. Preferably a closing plug 40 is provided in the lower face of the ram 16a. With this construction the gas which is supplied under pressure to conduit 26a escapes into the space below the ram upon withdrawal of the ram by passing from passages 25a around the edges of the lower end of the ram. The diameter of the lower end of the ram permits such gas flow. With the construction shown in Fig. 1 the diameter of the supplemental or dummy head is such as to provide for such gas flow upon upward withdrawal of the ram.

What I claim is:

1. The method of making metal sheathed cable which supplements the usual steps of the extrusion process by the step of introducing a special atmosphere into the extruding chamber while the press ram is in the chamber and is being withdrawn therefrom and by such special atmosphere at all times entirely preventing the introduction of free oxygen into the extrusion chamber to thereby preclude the oxidation of the metal during the step of filling the chamber with metal, and utilizing the special atmosphere to introduce lubricant into the chamber.

2. The method of making metal sheathed cable which supplements the usual steps of the extrusion process by the step of introducing a special atmosphere through the press ram and into the extruding chamber while the press ram is being withdrawn therefrom and by such special atmosphere at all times entirely preventing the introduction of free oxygen into the extrusion chamber to thereby preclude the oxidation of the metal during the step of filling the chamber with metal.

HORACE A. STAPLES.